# EUROPEAN PATENT SPECIFICATION

(11) **EP 1 904 314 B1**
(45) Date of publication and mention of the grant of the patent: **30.11.2011**
(21) Application number: 06741302.1
(22) Date of filing: 11.05.2006
(51) Int. Cl.: B43L 1/10, B43L 1/00

(54) **METHOD FOR MANUFACTURING A VISUAL COMMUNICATION PANEL HAVING A CERAMIC SURFACE LAYER**
VERFAHREN ZUR HERSTELLUNG EINER ANZEIGETAFEL MIT EINER KERAMISCHEN FLÄCHENSCHICHT
PROCÉDÉ DE FABRICATION D'UN PANNEAU DE COMMUNICATION VISUEL

(30) Priority: 13.05.2005 BE 200500244
(43) Date of publication of application: 02.04.2008
(73) Proprietor: Polyvision, Naamloze Vennootschap, 3600 Genk (BE)
(72) Inventor: GYPEN, Leo Albert Julia, B-3520 ZONHOVEN (BE)
(74) Representative: Donné, Eddy
(86) International application number: PCT/BE2006/000050
(87) International publication number: WO 2006/119592

(56) References cited:
- EP-A- 1 057 657
- WO-A-02/37409
- CH-A- 663 762
- DE-A- 1 629 512
- DE-A- 2 749 402
- DE-A- 2 756 908
- DE-C- 9 468
- US-A- 4 123 590

## Description

The present invention concerns a method for manufacturing a visual communication panel, in particular a panel with an porcelain or vitreous enamelled surface which is designed to be written on with dry, erasable felt-tip pens or to be used as a projection screen.

Known communication panels usually consist of a support made of a wood fibre board, a paper honeycomb structure or a synthetic onto which is fixed a metal plate having a coat of enamel on it, on the visible side of the panel.

The back of the panels is either or not provided with a supporting plate and/or a foil which can serve as a damp-proof guard.

A disadvantage of such panels is that the coat of enamel is usually relatively smooth and hence glares, in order to be easily wipeable for felt-tip pens, such that annoying light reflections may occur due to incident light of lamps, and as a result of which spectators can hardly or not see what is being written or projected on the panel.

Matt enamelled panels which are designed as a projection screen or as a board to be written on with dry, erasable felt-tip pens, have less annoying light reflections than their glossy variants, but they are more difficult to wipe in a dry manner.

Organic visual communication panels made of lacquered steel are usually far less scratch-resistant, wear-resistant and hence have a shorter life compared to the above-mentioned enamelled panels.

WO 02/37409 describes a method for manufacturing a porcelain enameled writing board. The aim is to obtain a writing board with determination of the position of the writing pen combined with the advantages offered by an enameled writing board.

DE 2.749.402 describes an alternative for an enameled writing board, in which the surface of the board is composed of a mixture of inorganic components and of hardenable organic resin which is hardened at a temperature of about 130 °C. This formulation allows a production of boards at a lower temperature, and with an enamel-like surface.

EP 1.057.657 describes a process for fabricating a writing board, and triers to prevent reflections by using a matted glass surface to write on. The matting of the glass is obtained by any known means, such as by chemical etching with acid such as hydrofluoric acid, or by sand blasting.

The present invention aims to remedy the above-mentioned and other disadvantages.

To this end, the invention concerns a method for manufacturing a visual communication panel which mainly consists of a support onto which is provided a coat of porcelain or vitreous enamel, whereby a sol-gel dispersion is provided on the visible side of the coat of porcelain or vitreous enamel which is then tempered in order to form a mainly glassy or ceramic cover layer that reduces the reflection of light by the porcelain or vitreous enamel.

An advantage of the method according to the invention is that it makes it possible to manufacture communication panels with a relatively large hardness and resistance to wear, possibly even much larger than that of the above-mentioned organic visual communication panels.

The above-mentioned dispersion preferably also contains particles of metal oxides in an order of magnitude which is larger than the wavelength of visible light.

This preferred method offers the additional advantage that the glare of the thus obtained communication panels is relatively low.

Indeed, by providing the above-mentioned particles in the cover layer on the coat of enamel, the incident light on the panel is diffused, such that the glare of the panel is reduced, and annoying light reflections of lamps are restricted.

According to yet another preferred method, the above-mentioned dispersion contains fluorine containing products.

Adding fluorine containing products to the above-mentioned dispersion offers the advantage that the surface tension of the finished cover layer is relatively low, as a result of which the ink of felt-tip pens can be removed relatively easily from the cover layer in a dry manner.

According to a further preferred method, the thickness of the sol-gel coat is designed to be equal to one fourth of the wavelength of visible light, resulting in a sol-gel thickness of between 75 and 180 nanometres.

In this way the sol-gel coat forms a quarter wavelength anti-reflection layer. Indeed, a first portion of the visible light that hits the communication panel is reflected by the external surface of the sol-gel coat, and a second portion of the visible light is reflected by the interface between the sol-gel coat and the porcelain or vitreous enamel. As the thickness of the sol-gel coat equals one fourth of the wavelength of visible light, both reflected waves are out of phase by 180° or π radians, and as a consequence they at least partially cancel each other.

By preference the sol-gel coating should have an index of refraction that is smaller than the index of refraction of the porcelain or vitreous enamel.

In order to better explain the characteristics of the present invention, the following preferred method according to the invention for manufacturing a visual communication panel is given as an example only without being limitative in any way, with reference to the sole accompanying figure 1, in which is represented a cross-section of a communication panel made according to a method of the invention.

Figure 1 represents a visual communication panel 1 which mainly consists of a support 2, onto which is fixed a metal or steel plate 3 which is provided with a coat of porcelain or vitreous enamel 4.

This coat of enamel 4 may consist of one or several layers, such as for example a first layer of enamel which adheres well to the above-mentioned metal plate or steel plate 3, and a top layer of enamel with the required properties such as for example a required colour.

The above-mentioned support 2, metal plate 3 and coat of enamel 4 are generally known in the domain of visual communication panels 1, and therefore they will not be further described in detail here.

According to the invention, a glassy or ceramic cover layer 5 with a thickness of preferably some 3 micrometers is provided on the above-mentioned coat of enamel 4.

This cover layer 5 is formed by providing what is called a sol-gel dispersion on the coat of enamel 4 and by subsequently tempering the dispersion at a temperature situated between 200° and 600°C, and which preferably amounts to some 510°C.

The above-mentioned sol-gel dispersion is hereby defined as a usually colloidal solution of inorganic metal salts and/or organic metal compounds, such as metal alcoxides, whereby this solution or, more particularly, liquid dispersion is transformed in what is called a 'sol' state during a drying process, and forms the above-mentioned cover layer 5 after some tempering.

The sol-gel dispersion is hereby preferably prepared from a basic solution of metal alcoxydes onto which are preferably added an aqueous colloidal silica solution and/or particles of metal oxide and/or fluorine containing products.

Examples of useful metal alcoxydes are among others: tetra methoxy silane [Si(OCH₃)₄]; tetra ethoxy silane [Si(OC₂H₅)₄]; methyl triethoxy silane [Si(OCH₃)(OC₂H₅)₃]; tetra ethoxy titanium [Ti(OC₂H₅)₄]; tetra propyl oxide titanium [Ti(OC₃H₇)₄]; tetra butoxy titanium [Ti(OC₄H₉)₄]; tetra propyl oxide zirconium [Zr(OC₃H₇)₄].

The above-mentioned colloidal silica solution consists of an aqueous dispersion with silicon oxide particles in an order of magnitude of 5 to 100 nm, whereas the above-mentioned particles of metal oxides have dimensions which are at least larger than the wavelength of visible light and which are preferably situated between 1 and 3 micrometers.

The above-mentioned particles of metal oxides, ordered here according to their increasing index of light refraction, consist for example of silicon oxide, zirconium oxide and/or titanium oxide.

A practical example of a useful basic solution consists of:
- 65 mole percent of methyl triethoxy silane;
- 15 mole percent of tetra ethoxy silane;
- 10 mole percent of tetra butyl ortho titanate; and
- 10 mole percent of tetra propyl zirconate.

By means of the above-mentioned basic solution, an above-mentioned sol-gel dispersion can be prepared which is composed of:
- 63 mass percent of the above-mentioned basic solution;
- 10 mass percent of colloidal silica solution (e.g. K40 of "Chemiewerk Bad Köstritz");
- 24 mass percent of particles of metal oxides, of which:
   - 16 mass percent of silicon oxide;
   - 4 mass percent of titanium oxide;
   - 4 mass percent of zirconium oxide; and
   - 3 mass percent of ammonium fluorine.

This sol-gel dispersion is subsequently provided on the above-mentioned coat of enamel 4, after which the dispersion is transformed in a solid gel or what is called a 'sol' under the influence of heat which, after a drying process at some 95°C and the tempering thereof up to 510°C, forms the required glassy or ceramic cover layer 5.

The above-mentioned sol-gel dispersion can be provided on the coat of enamel 4, for example by immersing the coat of enamel 4 in the dispersion; by spraying the dispersion over the coat of enamel 4; by means of silkscreen printing; by what is called roll coating.

It should be noted that the above-mentioned particles of metal oxides can be traced as such in the formed cover layer 5, and have a light-diffusing effect in there, such that annoying light reflections by the visual communication panel can be minimized.

The present invention is by no means limited to the above-described method; on the contrary, such a method according to the invention for manufacturing a visual communication panel with a mainly glassy or ceramic layer that reduces the reflection of light can be made according to different variants while still remaining within the scope of the invention as defined in the claims.

## Claims

1. Method for manufacturing a visual communication panel which mainly consists of a support (2) onto which is provided a coat of porcelain or vitreous enamel (4), **characterised in that** a sol-gel dispersion is provided on the visible side of the coat of porcelain or vitreous enamel (4) which is subsequently tempered so as to form a mainly glassy or ceramic cover layer (5) that reduces the reflection of light by the porcelain or vitreous enamel.

2. Method according to claim 1, **characterised in that** particles of metal oxides are distributed in the above-mentioned dispersion, having dimensions which are larger than the wavelength of visible light.

3. Method according to claim 2, **characterised in that** the above-mentioned particles are in an order of magnitude situated between 1 and 3 micrometers.

4. Method according to claim 2, **characterised in that** the above-mentioned particles consist of silicon oxide and/or zirconium oxide and/or titanium oxide.

5. Method according to claim 1, **characterised in that** the above-mentioned dispersion contains an amount of colloidal silica.

6. Method according to claim 5, **characterised in that** the above-mentioned colloidal silica consists of silicon oxide particles in an order of magnitude of 5 to 100 nanometres.

7. Method according to any one of the preceding claims, **characterised in that** the sol-gel dispersion contains fluorine containing products.

8. Method according to claim 1, **characterised in that** the tempering is done at a temperature between 200 and 600°C, and preferably up to 510°C.

9. Method according to any one of the preceding claims, **characterised in that** the thickness of the sol-gel coat is designed to be equal to one fourth of the wavelength of visible light, resulting in a sol-gel thickness of between 75 and 180 nanometres.

## Patentansprüche

1. Verfahren zur Herstellung einer visuellen Kommunikationstafel, welche im Wesentlichen aus einem Träger (2) besteht, worauf ein Überzug aus Porzellan oder Glasemaille (4) angebracht wird, **dadurch gekennzeichnet, dass** eine Sol-Gel-Dispersion an der sichtbaren Seite des Überzugs von Porzellan oder Glasemaille (4) angebracht wird, die anschließend getempert wird, um eine im Wesentlichen glasartige oder keramische Deckschicht (5) zu bilden, die die Lichtreflektion durch das Porzellan oder die Glasemaille reduziert.

2. Verfahren nach Anspruch 1, **dadurch gekennzeichnet, dass** Partikel aus Metalloxiden in der vorgenannten Dispersion verteilt sind, mit Abmessungen, die größer als die Wellenlänge sichtbaren Lichts sind.

3. Verfahren nach Anspruch 2, **dadurch gekennzeichnet, dass** die vorgenannten Partikel in einer Größenordnung sind, die zwischen 1 und 3 Mikrometern liegt.

4. Verfahren nach Anspruch 2, **dadurch gekennzeichnet, dass** die vorgenannten Partikel aus Siliziumoxid und/oder Zirkonoxid und/oder Titanoxid bestehen.

5. Verfahren nach Anspruch 1, **dadurch gekennzeichnet, dass** die vorgenannte Dispersion einen Anteil an kolloidalem Silika enthält.

6. Verfahren nach Anspruch 5, **dadurch gekennzeichnet, dass** das vorgenannte kolloidale Silika aus Siliziumoxidpartikeln in einer Größenordnung von 5 bis 100 Nanometern besteht.

7. Verfahren nach einem der vorgenannten Ansprüche, **dadurch gekennzeichnet, dass** die Sol-Gel-Dispersion fluorhaltige Produkte enthält.

8. Verfahren nach Anspruch 1, **dadurch gekennzeichnet, dass** das Tempern auf einer Temperatur zwischen 200 und 600°C und bevorzugt bis zu 510°C durchgeführt wird.

9. Verfahren nach einem der vorgenannten Ansprüche, **dadurch gekennzeichnet, dass** die Dicke des Sol-Gel-Überzugs so gestaltet ist, dass sie gleich einem Viertel der Wellenlänge sichtbaren Lichts ist, was zu einer Sol-Gel-Dicke von zwischen 75 und 180 Nanometern führt.

## Revendications

1. Procédé pour la fabrication d'un panneau de communication visuel qui est constitué à titre principal d'un support (2) sur lequel on procure une couche de porcelaine ou d'émail vitreux (4), **caractérisé en ce qu'**on procure une dispersion de type sol-gel sur le côté visible de la couche de porcelaine ou d'émail vitreux (4) que l'on soumet ensuite à un recuit pour obtenir une couche de revêtement principalement céramique ou vitreuse (5) qui réduit la réflexion de la lumière à l'intervention de la porcelaine ou de l'émail vitreux.

2. Procédé selon la revendication 1, **caractérisé en ce qu'**on distribue des particules d'oxydes métalliques dans la dispersion mentionnée ci-dessus, dont les dimensions sont supérieures à la longueur d'onde de la lumière visible.

3. Procédé selon la revendication 2, **caractérisé en ce que** les particules susmentionnées possèdent un ordre de grandeur qui se situe entre 1 et 3 µm.

4. Procédé selon la revendication 2, **caractérisé en ce que** les particules susmentionnées sont constituées d'oxyde de silicium et/ou d'oxyde de zirconium et/ou d'oxyde de titane.

5. Procédé selon la revendication 1, **caractérisé en ce que** la dispersion susmentionnée contient une quantité de silice colloïdale.

6. Procédé selon la revendication 5, **caractérisé en ce que** la silice colloïdale mentionnée ci-dessus est constituée par des particules d'oxyde de silicium possédant un ordre de grandeur de 5 à 100 nm.

7. Procédé selon l'une quelconque des revendications précédentes, **caractérisé en ce que** la dispersion sol-gel contient des produits fluorés.

8. Procédé selon la revendication 1, **caractérisé en ce que** le traitement de recuit est mis en oeuvre à une température entre 200 et 600 °C, et de préférence jusqu'à une température de 510 °C.

9. Procédé selon l'une quelconque des revendications précédentes, **caractérisé en ce que** l'épaisseur de la couche sol-gel est conçue pour être égale à un quart de la longueur d'onde de la lumière visible, si bien que l'on obtient une épaisseur du sol-gel entre 75 et 180 nm.
